# EUROPEAN PATENT SPECIFICATION

(11) **EP 1 149 155 B1**
(45) Date of publication and mention of the grant of the patent: **27.04.2005**
(21) Application number: 99905576.7
(22) Date of filing: 01.02.1999
(51) Int. Cl.: C11D 17/00, C11D 11/00, C11D 11/02

(54) **CATIONIC PARTICLE AND A PROCESS FOR MAKING THEREOF**
KATIONISCHES TEILCHEN UND VERFAHREN ZU SEINER HERSTELLUNG
PARTICULE CATIONIQUE ET PROCEDE DE FABRICATION CORRESPONDANT

(43) Date of publication of application: 31.10.2001
(73) Proprietor: THE PROCTER & GAMBLE COMPANY, Cincinnati, Ohio 45202 (US)
(72) Inventor: KANDASAMY, Manivannan, Kobe 658-0032 (JP); NAEMURA, Kenji, Hyogo 671-16 (JP); DUFTON, Daniel, James, Newcastle upon Tyne NE7 7BG (GB); ROBLES, Eric San Jose, Kobe 658-0027 (JP); DEDEYAN, Aram Armand, Newcastle upon Tyne NE7 7DX (GB)
(74) Representative: Brooks, Maxim Courtney
(86) International application number: PCT/US1999/002082
(87) International publication number: WO 2000/044874

(56) References cited:
- WO-A-98/13453

## Description

### FIELD

The present invention relates to a cationic surfactant particle, particulate detergent compositions containing such cationic particle, and a process for making thereof.

### BACKGROUND

Recently, there has been considerable interest within the detergent industry for laundry detergents which are "compact" and therefore, have low dosage volumes. To facilitate production of these so-called low dosage detergents, many attempts have been made to produce high bulk density detergents, for example with a density of 600 g/l or higher. The low dosage detergents are currently in high demand as they conserve resources and can be sold in small packages which are more convenient for consumers. However, the extent to which modem detergent products need to be "compact" in nature remains unsettled. In fact, many consumers, especially in developing countries, continue to prefer a higher dosage levels in their respective laundering operations. Consequently, there is a need in the art of producing modem detergent compositions for flexibility in the ultimate density of the final composition.

Currently, the relative amounts and types of materials subjected to processes in the production of detergent granules has been limited. For example, it has been difficult to attain high levels of surfactant in the resulting detergent composition, a feature which facilitates production of detergents in a more efficient manner. Cationic surfactants are a common surfactant as well as co-surfactant for use in detergent compositions and is commonly available in a liquid form. In general, detergent compositions will contain one or more types of surfactants which are designed to loosen and remove different types of soils and stains.

The international application WO 98/13453 discloses a particle comprising a water-soluble cationic surfactant, an ethoxylated cationic mono-/di-/polyamines and a carrier material, e.g. sodium aluminosilicate zeolite. The particle has a moisture content of less than 15 %, the ratio absorbing material to cationic surfactant 7:1 to 1:1, anionic surfactants can be present in a much smaller amount. The detergent composition comprising the cationic particles have a density between 600 and 1200 g/l, in particular e.g. 700 or 850 g/l. The agglomeration process comprises mixing/agglomerating the water-soluble cationic surfactant with the carrier material, alternatively the particles can be produced by a spray drying proces.

Based on the foregoing, there is a need for a cationic surfactant material which is in a form that is easily incorporated into particulate detergent compositions. None of the existing art provides all of the advantages and benefits of the present invention.

### SUMMARY

The present invention relates to a cationic particle containing an aqueous cationic surfactant solution adsorbed to a water-insoluble high absorbing material, wherein the finished cationic particle has at least 30 weight-% cationic surfactant active and wherein the cationic surfactant is a mono C₆-C₁₆ N-alkyl or alkenyl ammonium surfactant wherein the remaining N-positions are substituted by methyl, hydroxyethyl or hydroxypropyl groups. A process for making the cationic particle is also described herein. These and other features, aspects, and advantages of the present invention will become evident to those skilled in the art from a reading of the present disclosure.

### DETAILED DESCRIPTION

While this specification concludes with claims distinctly pointing out and particularly claiming that which is regarded as the invention, it is believed that the invention can be better understood through a careful reading of the following detailed description of the invention. In this specification, all percentages, ratios, and proportions are by weight, all temperatures are expressed in degrees Celsius, molecular weights are in weight average, and the decimal is represented by the point (.), unless otherwise indicated.

As used herein, "comprising" means that other steps and other ingredients which do not affect the end result can be added. This term encompasses the terms "consisting of" and "consisting essentially of".

The present invention relates to a cationic particle containing an aqueous cationic surfactant solution adsorbed to a water-insoluble high absorbing material. It is beneficial to have the cationic surfactant in a particulate form for various reasons, since cationic surfactants are commonly available in liquid solution form. For example, in processing particulate detergent compositions in non-tower processes, the liquid cationic surfactant may make the mixture during agglomeration sticky due to the excess moisture. In addition, the cationic particle can be made a higher active particle, as compared to its liquid form, which provides formula space when formulating a particulate detergent composition. In addition, the cationic particle of the present invention has good dispersion and solubility when used in the wash water.

The present invention also meets the aforementioned needs in the art by providing a cationic particle which can be used to produce a particulate detergent composition for flexibility in the ultimate density of the final composition.

As used herein, the term "mean residence time" refers to following definition: "mean residence time (hr) = mass (kg) / flow throughput (kg/hr)".

### Cationic surfactant solution

The cationic particle of the present invention contains an aqueous cationic surfactant solution. The cationic surfactant solution has at least 70% water, preferably from 40% to 60%, more preferably from 50% to 60%, by weight of the surfactant solution. The amount of cationic active in the aqueous cationic surfactant solution is at least 30%, preferably from 40% to 60%, more preferably from 40% to 50%.

The cationic surfactant is C₆-C₁₆ N-alkyl or alkenyl ammonium surfactants wherein remaining N positions are substituted by methyl, hydroxyethyl or hydroxypropyl groups.

Additionally, useful cationic surfactants include water-soluble quaternary ammonium compounds of the form R₄R₅R₆R₇N⁺X ⁻, wherein R₄ is alkyl having from 10 to 20, preferably from 12-18 carbon atoms, and R₅, R₆ , and R₇ are each C₁ to C₇ alkyl preferably methyl; X⁻ is an anion, e.g. chloride. Examples of such trimethyl ammonium compounds include C₁₂₋₁₄ alkyl trimethyl ammonium chloride and cocoalkyl trimethyl ammonium methosulfate.

Additional cationic surfactants is a cationic choline ester-type quat surfactant which are preferably water dispersible compounds having surfactant properties and comprise at least one ester (i.e. -COO-) linkage and at least one cationically charged group. Suitable cationic ester surfactants, including choline ester surfactants, have for example been disclosed in U.S. Patents Nos. 4,228,042, 4,239,660 and 4,260,529.

Furthermore preferred additional cationic ester surfactants are those having the formula: wherein R₁ is a C₅-C₃₁ linear or branched alkyl, alkenyl or alkaryl chain or M.N⁺(R₆R₇R₈)(CH₂)ₛ; X and Y, independently, are selected from the group consisting of COO, OCO, O, CO, OCOO, CONH, NHCO, OCONH and NHCOO wherein at least one of X or Y is a COO, OCO, OCOO, OCONH or NHCOO group; R₂, R₃, R₄, R₆, R₇ and R₈ are independently selected from the group consisting of alkyl, alkenyl, hydroxyalkyl, hydroxyalkenyl and alkaryl groups having from 1 to 4 carbon atoms; and R₅ is independently H or a C₁-C₃ alkyl group; wherein the values of m, n, s and t independently lie in the range of from 0 to 8, the value of b lies in the range from 0 to 20, and the values of a, u and v independently are either 0 or 1 with the proviso that at least one of u or v must be 1; and wherein M is a counter anion.

Preferably R₂, R₃ and R₄ are independently selected from CH₃ and -CH₂CH₂OH.

Preferably M is selected from the group consisting of halide, methyl sulfate, sulfate, and nitrate, more preferably methyl sulfate, chloride, bromide or iodide.

Preferred water dispersible cationic ester surfactants are the choline esters having the formula: wherein R₁ is a C₁₁-C₁₉ linear or branched alkyl chain.

Particularly preferred choline esters of this type include the stearoyl choline ester quaternary methylammonium halides (R¹=C₁₇ alkyl), palmitoyl choline ester quaternary methylammonium halides (R¹=C₁₅ alkyl), myristoyl choline ester quaternary methylammonium halides (R¹=C₁₃ alkyl), lauroyl choline ester quaternary methylammonium halides (R¹=C₁₁ alkyl), cocoyl choline ester quaternary methylammonium halides (R¹=C₁₁-C₁₃ alkyl), tallowyl choline ester quaternary methylammonium halides (R¹=C₁₅-C₁₇ alkyl), and any mixtures thereof.

The particularly preferred choline esters, given above, may be prepared by the direct esterification of a fatty acid of the desired chain length with dimethylaminoethanol, in the presence of an acid catalyst. The reaction product is then quaternized with a methyl halide, preferably in the presence of a solvent such as ethanol, propylene glycol or preferably a fatty alcohol ethoxylate such as C₁₀-C₁₈ fatty alcohol ethoxylate having a degree of ethoxylation of from 3 to 50 ethoxy groups per mole forming the desired cationic material. They may also be prepared by the direct esterification of a long chain fatty acid of the desired chain length together with 2-haloethanol, in the presence of an acid catalyst material. The reaction product is then quaternized with trimethylamine, forming the desired cationic material.

Other suitable cationic ester surfactants have the structural formulas below, wherein d may be from 0 to 20. In a preferred aspect these cationic ester surfactant are hydrolysable under the conditions of a laundry wash method.

Cationic surfactants useful herein also include alkoxylated quaternary ammonium (AQA) surfactant compounds (referred to hereinafter as "AQA compounds") having the formula: wherein R¹ is a linear or branched alkyl or alkenyl moiety containing from 8 to 18 carbon atoms, preferably 10 to 16 carbon atoms, most preferably from 10 to 14 carbon atoms; R² is an alkyl group containing from one to three carbon atoms, preferably methyl; R³ and R⁴ can vary independently and are selected from hydrogen (preferred), methyl and ethyl; X- is an anion such as chloride, bromide, methylsulfate, sulfate, sufficient to provide electrical neutrality. A and A' can vary independently and are each selected from C₁-C₄ alkoxy, especially ethoxy (i.e., -CH₂CH₂O-), propoxy, butoxy and mixed ethoxy/propoxy; p is from 0 to 30, preferably 1 to 4 and q is from 0 to 30, preferably 1 to 4, and most preferably to 4; preferably both p and q are 1. See also: EP 2,084, published May 30, 1979, by The Procter & Gamble Company, which describes cationic surfactants of this type which are also useful herein.

AQA compounds wherein the hydrocarbyl substituent R¹ is C₈-C₁₁, especially C₁₀, enhance the rate of dissolution of laundry granules, especially under cold water conditions, as compared with the higher chain length materials. Accordingly, the C₈-C₁₁ AQA surfactants may be preferred by some formulators. The levels of the AQA surfactants used to prepare finished laundry detergent compositions can range from 0.1% to 5%, typically from 0.45% to 2.5%, by weight.

According to the foregoing, the following are nonlimiting, specific illustrations of AQA surfactants used herein. It is to be understood that the degree of alkoxylation noted herein for the AQA surfactants is reported as an average, following common practice for conventional ethoxylated nonionic surfactants. This is because the ethoxylation reactions typically yield mixtures of materials with differing degrees of ethoxylation. Thus, it is not uncommon to report total EO values other than as whole numbers, e.g., "EO2.5", "EO3.5", and the like.

| Designation | R¹ | R² | ApR³ | A'qR⁴ |
|---|---|---|---|---|
| AQA-1 | C₁₂-C₁₄ | CH₃ | EO | EO |
| (also referred to as Coco Methyl E02) | | | | |
| AQA-2 | C₁₂-C₁₆ | CH₃ | (EO)₂ | EO |
| AQA-3 | C₁₂-C₁₄ | CH₃ | (EO)₂ | (EO)₂ |
| (Coco Methyl E04) AQA-4 | C₁₂ | CH₃ | EO | EO |
| AQA-5 | C₁₂-C₁₄ | CH₃ | (EO)₂ | (EO)₃ |
| AQA-6 | C₁₂-C₁₄ | CH₃ | (EO)₂ | (EO)₃ |
| AQA-7 | C₈-C₁₈ | CH₃ | (EO)₃ | (EO)₂ |
| AQA-8 | C₁₂-C₁₄ | CH₃ | (EO)₄ | (EO)₄ |
| AQA-9 | C₁₂-C₁₄ | C₂H₅ | (EO)₃ | (EO)₃ |
| AQA-10 | C₁₂-C₁₈ | C₃H₇ | (EO)₃ | (EO)₄ |
| AQA-11 | C₁₂-C₁₈ | CH₃ | (propoxy) | (EO)₃ |
| AQA-12 | C₁₀-C₁₈ | C₂H₅ | (iso-propoxy)₂ | (EO)₃ |
| AQA-13 | C₁₀-C₁₈ | CH₃ | (EO/PO)₂ | (EO)₃ |
| AQA-14 | C₈-C₁₈ | CH₃ | (EO)₁₅* | (EO)₁₅* |
| AQA-15 | C₁₀ | CH₃ | EO | EO |
| AQA-16 | C₈-C₁₂ | CH₃ | EO | EO |
| AQA-17 | C₉-C₁₁ | CH₃ | - EO 3.5 Avg. - | |
| AQA-18 | C₁₂ | CH₃ | - EO 3.5 Avg. - | |
| AQA-19 | C₈-C₁₄ | CH₃ | (ED)₁₀ | (EO)₁₀ |
| AQA-20 | C₁₀ | C₂H₅ | (EO)₂ | (EO)₃ |
| AQA-21 | C₁₂-C₁₄ | C₂H₅ | (EO)₅ | (EO)₃ |
| AQA-22 | C₁₂-C₁₈ | C₃H₇ | Bu | (EO)₂ |
| AQA-23 | C₈-C₁₀ | CH₃ | CH₃ | CH₂ CH₂OH |

| | | | | |
|---|---|---|---|---|
| *Ethoxy, optionally end-capped with methyl or ethyl. | | | | |

The preferred bis-ethoxylated cationic surfactants herein are available under the trade name ETHOQUAD from Akzo Nobel Chemicals Company.

Highly preferred bis-AQA compounds for use herein are of the formula wherein R¹ is C₁₀-C₁₈ hydrocarbyl and mixtures thereof, preferably C₁₀, C₁₂, C₁₄ alkyl and mixtures thereof, and X is any convenient anion to provide charge balance, preferably chloride. With reference to the general AQA structure noted above, since in a preferred compound R¹ is derived from coconut (C₁₂-C₁₄ alkyl) fraction fatty acids, R² is methyl and ApR³ and A'qR⁴ are each monoethoxy, this preferred type of compound is referred to herein as "CocoMeEO2" or "AQA-1" in the above list.

Other preferred AQA compounds herein include compounds of the formula: wherein R¹ is C₁₀-C₁₈ hydrocarbyl, preferably C₁₀-C₁₄ alkyl, independently p is 1 to about 3 and q is 1 to about 3, R² is C₁-C₃ alkyl, preferably methyl, and X is an anion, especially chloride.

Other compounds of the foregoing type include those wherein the ethoxy (CH₂CH₂O) units (EO) are replaced by butoxy (Bu), isopropoxy [CH(CH₃)CH₂O] and [CH₂CH(CH₃O] units (i-Pr) or n-propoxy units (Pr), or mixtures of EO and/or Pr and/or i-Pr units.

Additional cationic surfactants are described, for example, in the "Surfactant Science Series, Volume 4, Cationic Surfactants" or in the "Industrial Surfactants Handbook". Classes of useful cationic surfactants described in these references include amide quats (i.e., Lexquat AMG & Schercoquat CAS), glycidyl ether quats (i.e., Cyostat 609), hydroxyalkyl quats (i.e., Dehyquart E), alkoxypropyl quats (i.e., Tomah Q-17-2), polypropoxy quats (Emcol CC-9), cyclic alkylammonium compounds (i.e., pyridinium or imidazolinium quats), and/or benzalkonium quats.

### High absorbing material

The cationic particle of the present invention also contains a water-insoluble high absorbing material. The water-insoluble high absorbing material is a material having an oil absorption (using di-butyl phthalate) of preferably from 140 mL/100g to 400 mL/100g, even more preferably from 200 mL/100g to 300 mL/100g.

Preferably, the high absorbing material is selected from the group consisting of aluminosilicate, precipitated silica, amorphous silica, talc, and mixtures thereof.

Especially preferred are sodium aluminosilicates and amorphous precipitated silica. An example of an amorphous precipitated silica is a porous hydrophyllic silica (trademark SIPERNAT 22S) available by DeGussa. Another example of a precipitated silica is a white carbon, such as calcium silicate synthetic amorphous silica, (trademark Carplex) available by Shionogi and Company Ltd.

In a preferred cationic particle, the ratio of the high absorbing material to the cationic surfactant active when forming the particle is from 1:3 to 1:1, even more preferably from 1:2 to 1:1. Absorption here means that the high absorbing material is mixed and coated with the cationic surfactant solution, and/or that the high absorbing material is impregnated with the cationic surfactant solution.

The finished cationic particle has a mean particle size of greater than 100 microns, and preferably from 100 microns to 1000 microns, more preferably from 150 microns to 650 microns.

The finished cationic particle has the following composition, by weight percent of the cationic particle: cationic surfactant active at least 30%; and preferable from 30% to 65% cationic surfactant active, moisture content of from 3% to 15%, and the balance, the high absorbing material. Optionally filler and anionic surfactant may be included.

One embodiment for the cationic particle contain in addition, some anionic surfactant. If included, the ratio of anionic surfactant active to cationic surfactant active is from 1:10 to 1:30, preferably from 1:15 to 1:25. By weight percentage of the finished cationic particle, the content of anionic surfactant is preferably from 1 % to 5%. Of course, the anionic surfactant may in addition be included as an additional cleaning component for the final detergent composition. Although not wanting to be limited by theory, it is believed that the addition of small quantities of anionic surfactant in the cationic particle provides free flow characteristics to the cationic particle and provides a less sticky surface on the cationic particle.

The cationic particle optionally also contains a filler, such as soda ash, other silicate, and/or sulfate.

### Additional Detergent Composition Components

The cationic particle may be formulated in detergent compositions. Such detergent compositions herein may optionally comprise other known detergent cleaning components including alkoxylated polycarboxylates, bleaching compounds, brighteners, chelating agents, clay soil removal / anti-redeposition agents, dye transfer inhibiting agents, enzymes, enzyme stabilizing systems, fabric softeners, polymeric soil release agents, polymeric dispersing agents, suds suppressors. The detergent composition may also comprise other ingredients including carriers, hydrotropes, processing aids, dyes or pigments. The preferred detergent compositions have a wide range of density, e.g., from 300 g/l to 1000 g/l, especially for high dense detergent agglomerates e.g., from 600 g/l to 850 g/l.

The cationic particle can be used to formulate detergent compositions. In such detergent compositions, the amount of cationic particle, by weight of the final detergent composition is preferably from 0.5% to 30%, more preferably from 0.5% to 10%.

### Process

Preferred examples of the process of making the cationic particle of the present invention is described below. In one method of making the cationic particle via a spray drying process, the cationic surfactant solution, high absorbing material, and optionally anionic surfactant and a filler, are mixed and agitated to form a substantially homogenous mixture. The mixture is then sprayed into a tower, wherein cationic particles are formed. In another method of making the cationic particle via an agglomeration process, the cationic surfactant solution is added to the high absorbing material and agitated in a mixer to form a moist granular powder, or agglomerate for a mean residence time of from 1 to 10 min. The powder is then dried, such as in a fluid bed dryer, to form the finished cationic particle.

### EXAMPLES

The following examples further describe and demonstrate embodiments within the scope of the present invention.

In one embodiment, cationic surfactant solution (30-70% active), amorphous precipitated silica, optionally sodium carbonate, optionally sodium linear alkyl benzene sulfonate and water, are mixed in a crutcher tank mix. The mixture is then fed into the spray tower and cationic particles having about 150 microns are formed. The spray tower's drying temperature is about 160°C to 170°C.

In another embodiment, 100 kg/hr of amorphous precipitated silica is fed into a mixer, such as a Loedige KM mixer, and 250 kg/hr of cationic surfactant solution is added to the mixer at one or more points while mixing takes place. The calculated mean residence time in the mixer of the silica is 1-10 minutes. The moist granules from the mixer are then fed to a fluid bed dryer, where the moisture is removed by warm air at 100°C to 150°C, preferably 115°C to 130°C. The resultant cationic particles have a mean particle size of 100 to 1000 microns, preferably 350 to 650 microns. The finished agglomerate particle is free-flowing without the need for additional ingredients.

The following examples show cationic particle compositions of the present invention :

| Example | Ex.1 | Ex.2 | Ex.3 | Ex. 4 | Ex.5 |
|---|---|---|---|---|---|
| Cationic surfactant A (%) | 50 | 50 | 50 | - | - |
| Cationic surfactant B (%) | - | - | - | 50 | 50 |
| SIPERNAT 22S (%) | 35 | - | 35 | 40 | 35 |
| Carplex 80D (%) | - | 40 | - | - | - |
| NaLAS (%) | 2 | - | - | - | 2 |
| Soda Ash (%) | 8 | 5 | 10 | - | 8 |
| Water (%) | 5 | 5 | 5 | 10 | 5 |
| Cationic surfactant A = C12-14 Dimethyl Hydroxyethyl Ammonium Chloride Solution | | | | | |
| Cationic surfactant B = C8-10 Dimethyl Hydroxyethyl Ammonium Chloride Solution | | | | | |

It is understood that the examples and embodiments described herein are for illustrative purposes only and that various modifications or changes in light thereof will be suggested to one skilled in the art.

## Claims

1. A cationic particle, comprising an aqueous cationic surfactant solution adsorbed to a water-insoluble high absorbing material, wherein the finished cationic particle has at least 30% cationic surfactant active,
wherein the cationic surfactant is a mono C₆₋₁₆ N-alkyl or alkenyl ammonium surfactant wherein the remaining N positions ane substituted by methyl, hydroxyethyl or hydroxypropyl groups.

2. The cationic particle of Claim 1, wherein the high absorbing material has an oil absorption, using di-butyl phthalate, of from 140 mL100g to 400 mL/100g.

3. The cationic particle of Claim 2, wherein the ratio of the high absorbing material to the cationic surfactant active is from 1:3 to 1:1.

4. The cationic particle of Claim 2, wherein the high absorbing material is selected from the group consisting of aluminosilicate, precipitated silica, amorphous silica, talc, and mixtures thereof.

5. The cationic particle of Claim 2, wherein the finished cationic particle has a moisture content of from 3% to 15%, by weight.

6. The cationic particle of Claim 2, wherein the cationic particle further comprises an anionic surfactant at a ratio of anionic surfactant active to cationic surfactant active is from 1:10 to 1:30.

7. The cationic particle of Claim 2, wherein the finished cationic particle has from 30% to 65% cationic surfactant active, and wherein the high absorbing particle is precipitated silica and/or amorphous silica.

8. A detergent composition comprising the cationic particle of Claim 1, wherein the density of the detergent composition is from 300 g/l to 1000 g/l.

9. A process for making a cationic particle according to claim 1 comprising:
a. mixing an aqueous cationic surfactant solution and a water-insoluble high absorbing material, wherein the high absorbing material is coated with the cationic surfactant solution; and
b. spraying the mixture of (a) in a tower to form a cationic particle having a mean particle size of greater than 100 microns.

10. A process for making a cationic particle according to claim 1 comprising:
a. mixing an aqueous cationic surfactant solution and a water-insoluble high absorbing material in a mixer for a mean residence time of from 1 to 10 minutes in order to form agglomerates, and
b. drying the agglomerates of (a) in a dryer to form a cationic particle having a mean particle size of greater than 100 microns.

## Patentansprüche

1. Kationisches Teilchen, umfassend eine wässrige kationische Tensidlösung, die an ein wasserunlösliches, hoch absorbierendes Material adsorbiert ist, worin das fertige kationische Teilchen mindestens 30 % kationischen Tensidwirkstoff aufweist, worin das kationische Tensid ein Mono-C₆₋₁₆-N-Alkyl- oder -Alkenyl- ammoniumtensid ist, worin die verbleibenden N-Positionen durch Methyl-, Hydroxyethyl- oder Hydroxypropylgruppen substituiert sind.

2. Kationisches Teilchen nach Anspruch 1, worin das hoch absorbierende Material mit Hilfe von Dibutylphthalat eine Ölabsorption von 140 ml/100 g bis 400 ml/100 g aufweist.

3. Kationisches Teilchen nach Anspruch 2, worin das Verhältnis des hoch absorbierenden Materials zu dem kationischen Tensidwirkstoff von 1:3 bis 1:1 ist.

4. Kationisches Teilchen nach Anspruch 2, worin das hoch absorbierende Material ausgewählt ist aus der Gruppe, bestehend aus Alumosilicat, ausgefälltem Silica, amorphem Silica, Talk und Mischungen davon.

5. Kationisches Teilchen nach Anspruch 2, worin das fertige kationische Teilchen einen Feuchtigkeitsgehalt von 3 Gew.-% bis 15 Gew.-% aufweist.

6. Kationisches Teilchen nach Anspruch 2, worin das kationische Teilchen weiterhin ein anionisches Tensid in einem Verhältnis von anionischem Tensidwirkstoff zu kationischem Tensidwirkstoff von 1:10 bis 1:30 umfasst.

7. Kationisches Teilchen nach Anspruch 2, worin das fertige kationische Teilchen von 30 % bis 65 % kationischen Tensidwirkstoff aufweist und worin das hoch absorbierende Teilchen ausgefälltes Silica und/oder amorphes Silica ist.

8. Waschmittelzusammensetzung, umfassend das kationische Teilchen nach Anspruch 1, worin die Dichte der Waschmittelzusammensetzung von 300 g/l bis 1000 g/l ist.

9. Herstellungsverfahren für ein kationisches Teilchen nach Anspruch 1, umfassend:
a. Mischen einer wässrigen kationischen Tensidlösung und eines wasserunlöslichen, hoch absorbierenden Materials, worin das hoch absorbierende Material mit der kationischen Tensidlösung überzogen wird; und
b. Sprühen der Mischung von (a) in einen Turm, um ein kationisches Teilchen mit einer mittleren Teilchengröße von mehr als 100 µm zu bilden.

10. Herstellungsverfahren für ein kationisches Teilchen nach Anspruch 1, umfassend:
a. Mischen einer wässrigen kationischen Tensidlösung und eines wasserunlöslichen, hoch absorbierenden Materials in einem Mischer für eine mittlere Verweilzeit von 1 bis 10 Minuten, um Agglomerate zu bilden, und
b. Trocknen der Agglomerate von (a) in einem Trockner, um ein kationisches Teilchen mit einer mittleren Teilchengröße von mehr als 100 µm zu bilden.

## Revendications

1. Particule cationique, comprenant une solution tensioactive cationique aqueuse adsorbée sur une matière fortement absorbante insoluble dans l'eau, dans laquelle la particule cationique terminée a au moins 30 % d'agent tensioactif cationique actif, où l'agent tensioactif cationique est un agent tensioactif mono-N-alkyl- ou alkénylammonium en C₆ à ₁₆, dans lequel les positions N restantes sont substituées par des groupes méthyle, hydroxyéthyle ou hydroxypropyle.

2. Particule cationique selon la revendication 1, dans laquelle la matière fortement absorbante a un absorption d'huile, en utilisant le phtalate de dibutyle, allant de 140 ml/100 g à 400 ml/100 g.

3. Particule cationique selon la revendication 2, dans laquelle le rapport de la matière fortement absorbante sur l'agent tensioactif cationique actif est de 1/3 à 1/1.

4. Particule cationique selon la revendication 2, dans laquelle la matière fortement absorbante est choisie dans le groupe consistant en aluminosilicate, silice précipitée, silice amorphe, talc, et leurs mélanges.

5. Particule cationique selon la revendication 2, dans laquelle la particule cationique terminée a une teneur en humidité de 3 % à 15 %, en poids.

6. Particule cationique selon la revendication 2, dans laquelle la particule comprend de plus un agent tensioactif anionique dans un rapport de l'agent tensioactif anionique actif sur l'agent tensioactif cationique actif de 1/10 à 1/30.

7. Particule cationique selon la revendication 2, dans laquelle la particule terminée a de 30 % à 65 % d'agent tensioactif cationique actif, et dans laquelle la particule fortement absorbante est de la silice précipitée et/ou de la silice amorphe.

8. Composition détergente comprenant une particule cationique selon la revendication 1, dans laquelle la densité de la composition détergente est de 300 g/l à 1000 g/l.

9. Procédé de fabrication d'une particule cationique selon la revendication 1 comprenant:
a. le mélange d'une solution tensioactive cationique aqueuse et d'une matière fortement absorbante insoluble dans l'eau, dans laquelle la matière fortement absorbante est revêtue de solution tensioactive cationique; et
b. la pulvérisation du mélange (a) dans une tour pour former une particule cationique de taille moyenne supérieure ou égale à 100 µm.

10. Procédé de fabrication d'une particule cationique selon la revendication 1, comprenant:
a. le mélange d'une solution tensioactive cationique aqueuse et d'une matière fortement absorbante insoluble dans l'eau dans un mélangeur pendant un temps de séjour moyen de 1 à 10 minutes pour former des agglomérats, et
b. de séchage des agglomérats (a) dans un séchoir pour former une particule cationique de taille moyenne supérieure ou égale à 100 µm.
